# EUROPEAN PATENT SPECIFICATION

(11) **EP 0 082 514 B1**
(45) Date of publication and mention of the grant of the patent: **15.10.1986**
(21) Application number: 82111802.3
(22) Date of filing: 20.12.1982
(51) Int. Cl.: C25B 11/06, C25B 11/08, C25B 11/12, C25B 1/46

(54) **Electrode material**
Elektrodenmaterial
Matériau d'électrode

(30) Priority: 23.12.1981 US 333592; 23.12.1981 US 333593
(43) Date of publication of application: 29.06.1983
(73) Proprietor: THE DOW CHEMICAL COMPANY, Midland Michigan 48640-1967 (US)
(72) Inventor: McIntyre, James Arthur, Midland Michigan 48640 (US); Phillips, Robert Floyd, Michigan 48640 (US)
(74) Representative: Weickmann, Heinrich, Dipl.-Ing.

## Description

The invention resides in a particle suitable for use as an electrode material and a method for producing that material.

Chlorine and alkali metal hydroxide, for example, sodium hydroxide and potassium hydroxide, are commercially prepared by the electrolysis of the corresponding alkali metal chloride brines in an electrolytic cell. In one type of cell, where the anode is separated from the cathode by an ion permeable barrier, chlorine is evolved at the anode according to the reaction: while hydroxyl ions are produced at the cathode according to which is actually a multi-step reaction in which a hydrogen species is absorbed onto the surface of the cathode and the hydrogen molecule is desorbed therefrom.

The total hydrogen reaction, as a series of postulated adsorption and desorption steps, consumes about 0.8 volts in an alkaline solution, such that if the cathode in a chlorine cell is depolarized with oxygen instead of being allowed to evolve hydrogen, a savings of about 1.2 volts is possible, since the oxygen reduction reaction can theoretically generate 0.4 V. The cathodes previously developed for utilization of oxygen as a depolarizer were characterized by a structure of a thin sandwich of a microporous separator of plastic combined with a catalyzed layer, wet- proofed with, e.g., polytetrafluoroethylene, and pressed onto a wire screen current collector. In the prior art depolarized cathodes, oxygen is fed into the catalyst zone through the microporous backing. Such cathodes work. However, they suffered from various deficiencies, including separation or delamination of the various layers and flooding of the microporous layer.

US-A-4,292,197 discloses a method of preparing electroconductive, catalytic particles comprising the steps of: (a) forming a slurry of activated carbon and a thermally decomposable silver compound; (b) impregnating the activated carbon with the thermally decomposable silver compound; (c) drying the slurry whereby to form dried carbon product; (d) thereafter mixing the dried carbon product with a dispersion of a hydrophobic compound to form a second slurry; (e) impregnating the hydrophobic compound into the carbon product; (f) forming the second slurry into particles; and (g) thereafter heating the particles formed from the second slurry whereby to dry the particles, sinter the hydrophobic compound, and form electroconductive, catalytic, sintered particles having silver H0₂- disproportionation catalyst impregnated carbon and hydrophobic material.

The present invention resides in a particle suitable for use as an electrode material comprising a generally spherical substrate, a hydrophobic polymer and an electrochemically active, electrically conductive catalyst, characterized in that the substrate is selected from steel, iron, nickel, platinum, copper, silver or graphite, and is substantially completely coated with an admixture of a hydrophobic polymeric binder and an electrochemically active, electrically conductive catalyst selected from carbon black, activated carbon, platinum, silver or mixtures thereof, and wherein said particle has an average diameter of greater than 0.3 mm and less than 2.5 cm.

The invention also resides in a method for the production of the particles according to the invention characterized by forming a fluid admixture of an electrochemically active, electrically conductive catalyst selected from carbon black, activated carbon, platinum, silver or mixtures thereof, and a hydrophobic polymeric binder, bonding the coating to a generally spherical substrate selected from steel, iron, nickel, platinum, copper, silver or graphite by solidifying the fluid admixture, and forming the particles having an average diameter greater than 0.3 mm and up to 2.5 cm.

The invention further resides in a method of electrolyzing an aqueous electrolyte in an electrolytic cell having an anolyte compartment with an anode therein and a catholyte compartment with a cathode therein, which method comprises feeding said aqueous electrolyte to the cell, passing an electrical current between the anode and the cathode and recovering the products of electrolysis, at least one of the electrodes being formed of an electrode material comprising the particles according to the invention.

The invention also resides in an electrolytic cell having an anolyte compartment with an anode therein and a catholyte compartment with a cathode therein, means for feeding an aqueous electrolyte to the cell, means for passing an electrical current between the anode and the cathode, and means for recovering the products of electrolysis from the cell, at least one of the anode or cathode being formed of an electrode material comprising the particles according to the invention.

Optionally, the cell may contain an ion permeable barrier located between the anode and the cathode. Optionally, the cell may include a means to feed a gas to the electrode.

A bed of these particles has been found to be useful as a gas electrode. The electrode may be used as a cathode or as an anode.

The substrate, upon which a coating is applied, should be a material which will hold its shape. To provide for a convenient method of preparing the hereindescribed particles, the substrate is preferably a material which will not substantially deform when heated to a temperature of 350-375°C for a period of 1 hour.

The substrate may be a sintered material, a solid material, or a bonded agglomeration of small particles. The materials are selected from steel, iron, graphite, nickel, platinum, copper, and silver. Particularly preferred is graphite, because of its availability and its low cost.

The average diameter of the particle is greater than 0.3 mm and up to as large as 2.5 cm. This maximizes the surface area and gives a high porosity to the bed of particles. Particles having a size of from 0.7 mm to 4 mm are particularly preferred when the particles are used as an electrode material. Particles smaller than 0.3 mm tend to pack and offer a high resistance to fluid flow through the bed of particles. Substrates larger than 2.5 cm are not preferred because there is a minimum amount of surface area for electrical chemical reactions to occur.

The spherical particles used form a bed having optimum porosity and surface area. Irregularly shaped particles tend to pack and minimize the porosity of the bed.

The substrate need not be chemically inert to the electrolyte or the products of electrolysis of the process in which the particle is used. Preferably, however, the substrate is chemically inert so the coating need not totally cover the substrate. If the substrate is not chemically inert, the complete coating prevents reaction between the substrate and the electrolyte or the products of electrolysis.

The coating on the substrate is an admixture of a binder and an electrochemically active, electrically conductive catalyst. The binder should be a material which may be put into a fluid form by melting, dispersing, or dissolving. The binder should be chemically stable to any electrolyte or products it will contact when in use in an electrolytic cell. The binder should be firmly stable at the temperature of operation for the electrochemical cell in which it will be used. The binder need not itself be electrically conductive, since the catalyst mixed with it is electrically conductive. The coating may be a porous coating or a nonporous coating depending on the materials of construction of the substrate. If the substrate is chemically inert to the electrolyte, the coating may be a porous coating. If, however, the substrate is not chemically inert to the electrolyte, the coating should be nonporous to prevent reactions between the substrate and the electrolyte or electrolytic products from occurring.

The binder is a hydrophobic material. When used as an electrode material, the hydrophobic binder will cause bubbles to form on the surface of the particles and provides maximum contact between the gas and the liquid. If the binder is not hydrophobic, the surfaces of the particles will be wetted and no bubbles will form.

Various types of hydrophobic material may be used as a binder. The hydrophobic material may be a polyfluorocarbon, for example, polytetrafluoroethylene, polychlorotrifluoroethylene, poly- trifluoroethylene, polyvinylfluoride, polyvinylidene fluoride and copolymers, including interpolymers and terpolymers having tetrafluoroethylene, trifluoroethylene, chlorotrifluoroethylene, vinylidene fluoride and vinyl fluoride. Particularly preferred is polytetrafluoroethylene.

The particles also contain in the coating an electrochemically active, electrically conductive catalyst as defined in claim 1. The selection of the catalyst will depend upon the type of process to which the electrode material will be put. Examples of such processes include the reduction of oxygen and the oxidation of hydrogen. For the reduction of oxygen, the preferred catalysts include such things as carbon blacks, platinum, silver and activated carbon. Carbon black is particularly preferred because of its good physical characteristics and its availability. Preferred are carbon black catalysts having surface areas of from 100 to 1,000 square meters per gram of catalyst. Particularly preferred are those having a surface area from 150 to 500 square meters per gram of catalyst.

The substrate is substantially completely coated with the binder catalyst mixture, i.e. the coating covers substantially the entire surface of the particle. The coating may be of any convenient thickness. Thicknesses of about 1 mil (0,0254 mm) are particularly preferred. This provides an adequate coating to cover substantially the entire surface of the particle, yet is sufficiently thin to conserve the catalyst-binder mixture required to cover the particle. Thickness in excess of 5 to 6 mils (0,127-0,152 mm are wasteful in that a substantial portion of the catalyst is unavailable for reaction since it is covered by additional catalyst and binder.

Optionally, the coating may additionally include a peroxide decomposition catalyst.

The peroxide decomposition catalysts are known in the art and are typically transition metals having hydrogen adsorption properties. Preferred peroxide decomposition catalysts include copper, silver, platinum, gold, and mixtures or compounds thereof. Silver and platinum and mixtures or compounds thereof mixed with carbon black are especially preferred.

Another particularly desirable class of known peroxide decomposition catalysts are compounds of (1) alkali metals, alkaline earth metals, and metals of Group IIIB, with (2) transition metals, which compounds are further characterized by electrocatalytic or surface catalytic properties. Especially preferred are the perovskites.

The invention includes within its scope a method for the production of coated particles suitable for use as an electrode material. The coated particles are prepared by forming a fluid admixture of a particulated substrate, an electrochemically active, electrically conductive catalyst and a binder. The catalyst is bonded to the substrate by solidifying the fluid admixture. This forms a particle having a substrate coated with a binder and a catalyst.

The fluid admixture is initially formed by blending a particulated substrate with a catalyst and a binder. The admixture may be made fluid in one of several ways. The binder, itself, may be heated to a temperature at which it is softened or melted. It may be softened or melted prior to being mixed with the catalyst and the substrate or in situ with the catalyst and substrate.

An alternative method of forming the fluid admixture is to disperse the binder, catalyst and substrate in a liquid medium. Various liquid mediums which are nonreactive with the three components of the admixture may be used. Particularly preferred are water or other liquid materials which are not solvents for any of the components of the admixture. The dispersion may be made after the components have been admixed or any one of the components may be dispersed in a liquid prior to being blended with the other components. It is important to have the components adequately dispersed in the liquid medium.

A third way of forming the liquid admixture is to dissolve the binder in a solvent. The dissolved binder may then be admixed with the catalyst and the substrate. The solvent should not have the ability to dissolve neither the substrate nor the catalyst. The binder may be dissolved after or before the components have been blended.

After the fluid admixture has been formed, it is solidified to bond the coating to the substrate. The admixture may be solidified in one of several different ways. The solidification method is somewhat dependent upon the method initially used to form the fluid admixture. If the fluid admixture was formed by melting or softening the binder, mere cooling of the admixture will cause the binder to solidify. If the fluid admixture was formed by dispersing one or more of the components into a liquid medium, solidification may be caused by removing the liquid medium from the admixture. The liquid medium may be removed by heating the admixture to evaporate the liquid medium or by subjecting the admixture to a vacuum to vaporize the liquid medium. If the method used to form the liquid admixture was dissolving the binder in a solvent, solidification may be accomplished by removing the solvent. The solvent may be removed by heating to vaporize the solvent, by vacuum to remove the solvent, or by reacting the solvent with another component.

Optionally, the admixture, during solidification may be treated in a manner to prevent the coated particles from adhering together to form one, single mass. Agitation is a convenient way to prevent the particles from adhering to each other during the solidification process. The amount and severity of agitation used is minimal and can be accomplished by merely stirring or rolling the material during solidification. Agitation during solidification also helps enhance the uniformity of the coating onto the substrate.

Optionally, after solidification, the coated particles may be heated to a temperature near or above the softening point of the binder to enhance the bonding of the material to the substrate. Heating to this temperature causes the binder to soften and become more intermixed with the catalyst and better bonded to the substrate.

Optionally, the steps of coating the particle may be repeated a plurality of times. In this manner, the amount and thickness of the coating may be controlled depending on the number of times the process is repeated. The thickness of the coating is not critical to the invention.

Optionally, a surfactant may be added to the fluid admixture to enhance wetting of the substrate and the catalyst by the binder. This assures better contact and a more even distribution of the admixture. It is preferred that a type of surfactant be used that may be removed from the particle after the bonding has occurred. This is preferred because, when in use as an electrode material, the coated particle preferably is not wetted by the electrolyte. As was discussed earlier, the formation of gas bubbles on the surface of the particle is desired. The presence of a surfactant at this point would minimize the formation of gas bubbles since the wetting of the particles by an electrolyte would be enhanced. As a result, the preferred surfactants are the non-ionic surfactants which may be thermally decomposed leaving only a carbon residue. Such surfactants are well-known in the art and need no further elaboration.

Optionally, the particles may be washed after bonding to remove any catalyst which has not been bonded to the substrate. Water and other liquids which are not solvents for any of the components of the coating are suitable. Water is particularly preferred because of its convenience.

The weight or volume ratio of the catalyst and binder to the substrate depends on the degree of coating desired on the substrate. If a thin coating is desired, obviously only a small amount of catalyst and binder should be blended with the substrate to form a fluid admixture. Conversely, if a thick coating is desired, the amount of catalyst and binder should be increased.

The ratio of the amount of catalyst to the amount of binder may be varied over a rather wide range. For example, if carbon black is used as the catalyst, and polytetrafluoroethylene is used as the binder, weight ratios of from 4:1 to 1:4 may be used. Preferred ratios of carbon black to PTFE are from 1:1.5 to 1.5:1 by weight. Other catalyst and binders should also be used within this same general ratio.

If a metal powder is used as the catalyst, such as silver, platinum or other metals, it is convenient to express the proportion in terms of volume as opposed to weight. The metal powder to binder may be in the range of from 4:1 to 1:4, by volume. Preferably, the ratio should be from 1:1.5 to 1.5:1, by volume.

Optionally, various types of additional catalysts may be added to the fluid admixture. One of the preferred embodiments of the herein-described invention includes the addition of a peroxide decomposition catalyst, in conjunction with a carbon black catalyst. When both of these types of catalyst are used from 1 to 35 weight percent of the total catalyst used should be a peroxide decomposition catalyst and from 65 to 99 percent of the total amount of catalyst used should be the carbon black catalyst. Preferably, from 3 to 10 percent of the catalyst should be the peroxide decomposition catalyst and from 90 to 97 percent of the catalyst should be the carbon black catalyst. This catalyst mixture should be used in the ratios discussed earlier concerning the catalyst to binder ratio.

Commonly, the peroxide decomposition catalyst used to form the fluid admixture is a precursor catalyst. In other words, the material used in the fluid admixture is a compound of the catalyst, which must be thermally or chemically decomposed in order to form the catalyst itself. This thermal or chemical decomposition may be accomplished at any stage of the process of forming the coated particles. Preferably, the material is thermally or chemically decomposed prior to being mixed with the binder and the substrate. This allows better control of the thermal or chemical decomposition of the catalyst precursor. Additionally, it provides the maximum contact between the carbon black and the peroxide decomposition catalyst. If the two are blended and decomposed prior to being mixed with the substrate and the binder, maximum contact is obtained between the carbon black and the peroxide decomposition catalyst.

The herein-described coated particles are suitable for use as an electrode material, since they are electrically conductive and catalytically active. Conveniently, they may be used as a packed bed electrode. As such, they are formed into a bed and supported in some convenient manner within the cell. They are electrically connected with a power supply associated with the cell. Optionally, a current collector may be used. The current collector may be a wire mesh bag, wire mesh container or the like, surrounding the catalyzed particles and containing them therein.

If the coated particles include a peroxide decomposition catalyst, the particles may be used in a cell to produce a hydroxide. If the coated particles do not contain a peroxide decomposition catalyst, the particles may be used in a cell to produce a peroxide.

According to a preferred embodiment of the method of using the herein-described particles, an aqueous alkali metal halide brine is fed to an electrolytic cell having an anolyte compartment with an anode therein, and a catholyte compartment with cathode means therein, and, optionally an ion permeable barrier therebetween. Typically, the anode is a valve metal, for example, titanium, tantalum, tungsten, columbium, or the like, with a suitable electrocatalytic surface thereon. Suitable anodic electrocatalytic surfaces are well known in the art and include transition metals, oxides of transition metals, compounds of transition metals, especially platinum group metals, oxides of platinum group metals and compounds of platinum group metals. Especially preferred are compounds of oxides of platinum group metals with oxides of the valve metals, that is, titanium, tantalum, tungsten, columbium and the like.

The ion permeable barrier may be an electrolyte permeable diaphragm, for example, a deposited asbestos diaphragm, a preformed asbestos diaphragm, or a microporous synthetic diaphragm. Alternatively, the ion permeable barrier may be ion permeable but electrolyte impermeable as a cation selective permionic membrane. Typically, cation selective permionic membranes are fluorocarbon polymers having pendent acid groups thereon. Typical pendent acid groups include sulfonic acid groups, carboxylic acid groups, phosphonic acid groups, phosphoric acid groups, precursors thereof, and reaction products thereof.

The anolyte liquor is typically an aqueous brine containing from 120 to 250 grams per liter of sodium chloride or from 180 to 370 grams per liter of potassium chloride, and is typically at a pH of from 1.5 to 5.5. The brine feed is typically a saturated or substantially saturated brine, containing from 300 to 325 grams per liter of sodium chloride or from 450 to 500 grams per liter of potassium chloride. The catholyte liquor recovered from the electrolytic cell may be a catholyte liquor containing approximately 10 to 12 weight percent sodium hydroxide and 15 to 25 weight percent sodium chloride, or approximately 15 to 20 weight percent potassium hydroxide and approximately 20 to 30 weight percent potassium chloride, as where an electrolyte permeable barrier is utilized. Alternatively, the catholyte product may contain from 10 to 45 weight percent sodium hydroxide, or from 15 to 65 weight percent potassium hydroxide, as where the ion permeable barrier is a cation selective permionic membrane interposed between the anode and the cathode.

An oxidant, for example, oxygen, air or oxygen-enriched air, is preferably fed to the catholyte compartment as an electrical current is fed from the cathode compartment to the anode compartment, to provide an anode product of chlorine and a cathode product of alkali metal hydroxide, characterized by the substantial absence of gaseous hydrogen product. The invention is particularly directed to a preferred packed bed cathode including coated particles as herein described.

According to a further exemplification of the invention, there is provided an electrolytic cell having an anolyte compartment fabricated of a material resistant to concentrated, chlorinated alkali metal chloride brines, an anode in the anolyte compartment, a catholyte compartment that is fabricated of a material resistant to concentrated alkali metal hydroxide solutions, cathode means in said cathode compartment, and an ion permeable barrier interposed between the anode and the cathode means. The electrolytic cell herein contemplated is characterized by the catholyte compartment having means for feeding an oxidant to the electrolyte within the cathode compartment and cathode means which comprise individual particles of the invention.

In another preferred embodiment of the method of using the herein described particles to produce a peroxide aqueous hydroxide solution is fed to the electrolytic cell already described except no ion exchange membrane is used. The anolyte feed is typically an aqueous solution containing from 15 to 100 grams per liter of sodium hydroxide. The catholyte liquor recovered from the electrolytic cell may be a catholyte liquor containing approximately 0.5 to 3 weight percent hydrogen peroxide and 15 to 100 grams per liter sodium hydroxide.

As herein contemplated, an oxidant, for example, oxygen, air or oxygen-enriched air, is fed to the catholyte compartment as an electrical current is fed from the cathode compartment to the anode compartment, whereby to provide an anode product of oxygen and water and a cathode product of an alkali metal hydroxide and a peroxide, characterized by the substantial absence of gaseous hydrogen product. The invention is particularly directed to the cathode means for carrying out the reaction, which cathode means comprise coated particles as herein described.

According to a further exemplification of the invention, there is provided an electrolytic cell having an anolyte compartment fabricated of a material resistant to concentrated, alkali metal hydroxide solutions, an anode in the anolyte compartment, a catholyte compartment that is fabricated of a material resistant to concentrated alkali metal hydroxide solutions, cathode means in said cathode compartment, and an ion permeable barrier interposed between the anode and the cathode means. The electrolytic cell herein contemplated is characterized by the catholyte compartment having means for feeding an oxidant to the electrolyte within the cathode compartment and cathode means which comprise individual particles of the invention.

### Example 1

To prepare a catalytically active coating, 0.7 gram of carbon black was blended with 20 milliliters of an aqueous silver acetate solution having a concentration of 10 grams of silver acetate per liter of solution. A drop of surfactant (Triton@ X-100 a product manufactured by Rohm and Haas Co.) was added to enhance the wetting of the carbon black. The mixture was then oven dried at about 100°C. Thereafter, the mixture was heated for 1 hour at 350°C in a nitrogen atmosphere to thermally decompose the silver acetate. This material was then blended with 3.5 grams of a 1:10 aqueous emulsion (1 part Teflon@ 30B, a product manufactured by E. I. duPont de Nemours & Co., fluoropolymer to 10 parts water). A slurry was formed therebetween. To the slurry, 10 grams of 10 to 20 U.S. Mesh (0,84-2,00 mm) graphite particles were added.

### @ Trademark

After mixing, the material was dried at about 100°C. Thereafter, the material was heated for 1 hour at 350°C in a nitrogen atmosphere. The particles produced were graphite particles having a carbon-fluorocarbon-silver coating on their surfaces.

### Example 2

An electrolytic cell was assembled as described herein. The cell had an anode and a cathode separated by a porous asbestos diaphragm. The cathode was a packed bed of the particles produced in Example 1. The anode was ruthenium oxide coated titanium.

A sodium chloride brine solution having a concentration of about 300 grams per liter of NaCI was flowed into a compartment containing the anode. Oxygen gas was flowed into the openings between the particles comprising the cathode. Electrical current at a voltage of about 2 volts and at a current density of about 1 amp per square inch (0,155 A/cm²), was passed between the anode and the cathode to cause electrolysis of the brine solution to occur. Chlorine gas was produced at the anode and sodium hydroxide was produced at the cathode.

## Claims

1. A particle suitable for use as an electrode material comprising a generally spherical substrate, a hydrophobic polymer and an electrochemically active, electrically conductive catalyst, characterized in that the substrate is selected from steel, iron, nickel, platinum, copper, silver or graphite, and is substantially completely coated with an admixture of a hydrophobic polymeric binder and an electrochemically active, electrically conductive catalyst selected from carbon black, activated carbon, platinum, silver or mixtures thereof, and wherein said particle has an average diameter of greater than 0.3 mm and less than 2.5 cm.

2. The electrode material of Claim 1 characterized in that the substrate is selected from a sintered material, a solid material or a bonded agglomeration of small particles.

3. The particle of Claim 1 or 2, characterized in that the catalyst has a surface area of from 100 to 1000 m²jg of catalyst.

4. The particle of Claim 3, characterized in that the catalyst is an oxygen reaction catalyst.

5. The particle of Claim 4, characterized in that the catalyst is carbon black and has a surface area from 150 to 500 m²/g of catalyst.

6. The particle of Claim 3, characterized in that the catalyst is a peroxide decomposition catalyst selected from silver and platinum and mixtures or compounds thereof mixed with carbon black.

7. The particle of any one of the preceding claims, characterized in that the particle has an average diameter of from 0.7 mm to 4 mm, and said coating has a thickness of from 25 to 125 microns.

8. The particle of any one of the preceding claims characterized in that the hydrophobic polymeric binder is a polyfluorocarbon binder.

9. The particle of any one of claims 1 to 5, 7 or 8, characterized in that the catalyst is carbon black and the binder is polytetrafluoroethylene, and wherein the weight ratio of carbon black to binder is from 4:1 to 1:4, preferably from 1:1,5 to 1,5:1.

10. A method for the production of particles suitable for use as an electrode material according to any of claims 1 to 9 characterized by forming a fluid admixture of an electrochemically active, electrically conductive catalyst selected from carbon black, activated carbon, platinum, silver or mixtures thereof, and a hydrophobic polymeric binder, coating a generally spherical substrate selected from steel, iron, nickel, platinum, copper, silver or graphite with said admixture, solidifying the same, and forming the particles having an average diameter greater than 0.3 mm and up to 2.5 cm.

11. The method of Claim 10 characterized by forming the fluid admixture by heating the polymeric binder to a temperature at least as high as its softening temperature, and cooling the admixture to a temperature below the softening temperature to bond the coating to the substrate.

12. The method of Claim 10 characterized by forming the fluid admixture by dispersing the catalyst, binder and substrate in a liquid, and heating the admixture to evaporate the liquid to bond the coating to the substrate.

13. The method of any of Claims 10 to 12 characterized by forming the fluid admixture by dissolving the binder in a solvent, and heating the admixture to evaporate the solvent to bond the coating to the substrate.

14. The method of any of Claims 10 to 13 characterized in that the catalyst is carbon black and the binder is polytetrafluoroethylene, and wherein the weight ratio of carbon black to binder is from 4:1 to 1:4, preferably from 1:1,5 to 1,5:1.

15. The method of any of Claims 10 to 13 characterized in that if a metal powder is used as the catalyst the ratio of catalyst to binder is in the range of from 4:1 to 1:4 by volume, preferably in the range of from 1:1,5 to 1,5:1 by volume.

16. The method of any of Claims 10 to 15 characterized by adding a surfactant, preferably a non-ionic surfactant, to the admixture.

17. The method of any of Claims 10 to 16 characterized by adding a second catalyst which is a peroxide decomposition catalyst.

18. The method of Claim 17 wherein the total amount of catalyst in the admixture is from 1 to 35 weight percent peroxide decomposition catalyst and from 65 to 99 weight percent carbon black, and preferably from 3 to 10 and from 90 to 97 weight percent.

19. A method of electrolyzing an aqueous electrolyte in an electrolytic cell having an anolyte compartment with an anode therein and a catholyte compartment with a cathode therein, which method comprises feeding said aqueous electrolyte to the cell, passing an electrical current between the anode and the cathode and recovering the products of electrolysis, characterized in that at least one of the electrodes is formed of an electrode material comprising a plurality of packed particles according to any one of claims 1 to 9.

20. The method of Claim 19 characterized by positioning an ion permeable barrier between the anode and the cathode.

21. The method of Claim 19 or 20, characterized by feeding an oxygen containing gas to the cathode.

22. An electrolytic cell having an anolyte compartment with an anode therein and a catholyte compartment with a cathode therein, means for feeding an aqueous electrolyte to the cell, means for passing an electrical current between the anode and the cathode, and means for recovering the products of electrolysis from the cell, characterized in that at least one of the anode or cathode is formed of an electrode material comprising a plurality of packed particles according to any one of claims 1 to 18.

23. The cell of Claim 22 characterized in that the substrate comprises graphite, the catalyst is selected from carbon black, silver or platinum, and the hydrophobic binder material is polytetrafluoroethylene.

24. The cell of Claim 22 characterized in that the catalyst is a mixture of carbon black and a peroxide decomposition catalyst.

## Patentansprüche

1. Ein zur Verwendung als Elektrodenmaterial geeignetes Teilchen mit einem im allgemeinen kugelförmigen Substrat, einem hydrophoben Polymeren und einem elektrochemisch aktiven, elektrisch leitenden Katalysator, dadurch gekennzeichnet, daß das Substrat ausgewählt ist aus Stahl, Eisen, Nickel, Platin, Kupfer, Silber oder Graphit, und im wesentlichen vollständig mit einer Mischung eines hydrophoben polymeren Binders und einem elektrochemisch aktiven, elektrisch leitenden Katalysator ausgewählt aus Ruß, Aktivkohle, Platin, Silber oder Mischungen davon beschichtet ist, und worin das Teilchen einen mittleren Durchmesser von größer als 0,3 mm und kleiner als 2,5 cm besitzt.

2. Elektrodenmaterial nach Anspruch 1, dadurch gekennzeichnet, daß das Substrat ausgewählt ist aus einem gesinterten Material, einem festen Material oder einem gebundenen Agglomerat kleiner Teilchen.

3. Teilchen nach Anspruch 1 oder 2, dadurch gekennzeichnet, daß der Katalysator eine Oberfläche von 100 bis 1000 m²/g Katalysator besitzt.

4. Teilchen nach Anspruch 3, dadurch gekennzeichnet, daß der Katalysator ein Sauerstoffreaktionskatalysator ist.

5. Teilchen nach Anspruch 4, dadurch gekennzeichnet, daß der Katalysator Ruß ist und eine Oberfläche von 150 bis 500 m/g Katalysator besitzt.

6. Teilchen nach Anspruch 3, dadurch gekennzeichnet, daß der Katalysator ein Peroxidzersetzungs-Katalysator ist, ausgewählt aus Silber und Platin und Mischungen oder Verbindungen davon, gemischt mit Ruß.

7. Teilchen nach einem der vorhergehenden Ansprüche, dadurch gekennzeichnet, daß das Teilchen einen mittleren Durchmesser von 0,7 mm bis 4 mm besitzt und die Beschichtung eine Dicke von 25 bis 125 11m besitzt.

8. Teilchen nach einem der vorhergehenden Ansprüche, dadurch gekennzeichnet, daß der hydrophobe polymere Binder ein Polyfluorkohlenstoff-Binder ist.

9. Teilchen nach einem der Ansprüche 1 bis 5, 7 oder 8, dadurch gekennzeichnet, daß der Katalysator Ruß ist und der Binder Polytetrafluorethylen, und worin das Gewichtsverhältnis von Ruß zu Binder 4:1 bis 1:4, vorzugsweise 1:1,5 bis 1,5:1 beträgt.

10. Verfahren zur Herstellung von zur Verwendung als Elektrodenmaterial geeigneten Teilchen gemäß einem der Ansprüche 1 bis 9, dadurch gekennzeichnet, daß man eine fluide Mischung eines elektrochemisch aktiven, elektrisch leitenden Katalysators, ausgewählt aus Ruß, Aktivkohle, Platin, Silber oder Mischungen davon, und eines hydrophoben polymeren Binders bildet, ein im allgemeinen kugelförmiges Substrat ausgewählt aus Stahl, Eisen, Nickel, Platin, Kupfer, Silberoder Graphit mit dieser Mischung beschichtet, diese verfestigt, und die Teilchen mit einem mittleren Durchmesser von größer als 0,3 mm und bis zu 2,5 cm bildet.

11. Verfahren nach Anspruch 10, dadurch gekennzeichnet, daß man die fluide Mischung durch Erhitzen des polymeren Binders auf eine Temperatur bildet, die mindestens so hoch ist wie seine Erweichungstemperatur, und die Mischung auf eine Temperatur unterhalb der Erweichungstemperatur abkühlt, um die Beschichtung an das Substrat zu binden.

12. Verfahren nach Anspruch 10, dadurch gekennzeichnet, daß man die fluide Mischung durch Dispersion des Katalysators, Binders und Substrats in einer Flüssigkeit bildet, und die Mischung erhitzt, um die Flüssigkeit zu verdampfen, um die Beschichtung an das Substrat zu binden.

13. Verfahren nach einem der Ansprüche 10 bis 12, dadurch gekennzeichnet, daß man die fluide Mischung durch Lösen des Binders in einem Lösungsmittel bildet, und die Mischung erhitzt, um das Lösungsmittel zu verdampfen, um die Beschichtung an das Substrat zu binden.

14. Verfahren nach einem der Ansprüche 10 bis 13, dadurch gekennzeichnet, daß der Katalysator Ruß und der Binder Polytetrafluorethylen ist, und worin das Gewichtsverhältnis von Ruß zu Binder 4:1 bis 1:4, vorzugsweise 1:1,5 bis 1,5:1 ist.

15. Verfahren nach einem der Ansprüche 10 bis 13, dadurch gekennzeichnet, daß, wenn ein Metallpulver als Katalysator verwendet wird, das Volumenverhältnis von Katalysator zu Binder im Bereich von 4:1 bis 1:4, vorzugsweise im Bereich von 1:1,5 bis 1,5:1 liegt.

16. Verfahren nach einem der Ansprüche 10 bis 15, dadurch gekennzeichnet, daß man zur Mischung ein oberflächenaktives Mittel, vorzugsweise ein nichtionisches oberflächenaktives Mittel, zugibt.

17. Verfahren nach einem der Ansprüche 10 bis 16, dadurch gekennzeichnet, daß man einen zweiten Katalysator zugibt, der ein Peroxidzersetzungs-Katalysator ist.

18. Verfahren nach Anspruch 17, dadurch gekennzeichnet, daß die Gesamtmenge des Katalysators in der Mischung aus 1 bis 35 Gew.% Peroxidzersetzungs-Katalysator und 65 bis 99 Gew.% Ruß besteht, und vorzugsweise aus 3 bis 10 und 90 bis 97 Gew.%.

19. Verfahren zur Elektrolyse eines wässrigen Elektrolyts in einer elektrolytischen Zelle mit einem Anolytraum mit einer Anode und einem Katholytraum mit einer Kathode, durch Einspeisen des wässrigen Elektrolyten in die Zelle, Hindurchleiten eines elektrischen Stromes zwischen der Anode und der Kathode, und Gewinnung der Elektrolyseprodukte, dadurch gekennzeichnet, daß mindestens eine der Elektroden aus einem Elektrodenmaterial gebildet ist, das eine Vielzahl von gepackten Teilchen nach einem der Ansprüche 1 bis 9 enthält.

20. Verfahren nach Anspruch 19, dadurch gekennzeichnet, daß man zwischen der Anode und der Kathode eine ionenpermeable Trennschicht anbringt.

21. Verfahren nach Anspruch 19 oder 20, dadurch gekennzeichnet, daß man ein Sauerstoff enthaltendes Gas zur Kathode einführt.

22. Elektrolytische Zelle mit einem Anolytraum mit einer Anode und einem Katholytraum mit einer Kathode, Mittel zur Einspeisung eines wässrigen Elektrolyten in die Zelle, Mittel zum Hindurchleiten eines elektrischen Stromes zwischen der Anode und der Kathode, und Mittel zur Gewinnung der Elektrolyseprodukte aus der Zelle, dadurch gekennzeichnet, daß mindestens eine der Elektroden (Anode oder Kathode) aus einem Elektrodenmaterial gebildet ist, das eine Vielzahl von gepackten Teilchen nach einem der Ansprüche 1 bis 18 enthält.

23. Zelle nach Anspruch 22, dadurch gekennzeichnet, daß das Substrat Graphit umfaßt, der Katalysator ausgewählt ist aus Ruß, Silber oder Platin, und das hydrophobe Bindermaterial Polytetrafluorethylen ist.

24. Zelle nach Anspruch 22, dadurch gekennzeichnet, daß der Katalysator eine Mischung aus Ruß und einem. Peroxidzersetzungs-Katalysator ist.

## Revendications

1. Particule convenant pour être utilisée en tant que matériau d'électrode, comprenant un support sensiblement sphérique, un polymère hydrophobe et un catalyseur électriquement conducteur et électrochimiquement actif, caractérisée en ce que le support est choisi parmi l'acier, le fer, le nickel, le platine, le cuivre, l'argent ou le graphite et est sensiblement complètement revêtu d'un mélange d'un liant polymère hydrophobe et d'un catalyseur électriquement conducteur et électrochimiquement actif choisi parmi le noir de carbone, le charbon actif, le platine, l'argent ou des mélanges de ceux-ci, ladite particule ayant un diamètre moyen supérieur à 0,3 mm et inférieur à 2,5 cm.

2. Matériau d'électrode de la revendication 1, caractérisé en ce que le support est choisi parmi un matériau fritté, un matériau plein ou une agglomération liée de petites particules.

3. Particule de la revendication 1 ou 2, caractérisée en ce que le catalyseur présente une surface spécifique allant de 100 à 1000 m²/g de catalyseur.

4. Particule de la revendication 3, caractérisée en ce que le catalyseur est un catalyseur de réaction d'oxygène.

5. Particule de la revendication 4, caractérisée en ce que le catalyseur est du noir de carbone et présente une surface spécifique allant de 150 à 500 m^{z}/g de catatyseur.

6. Particule de la revendication 3, caractérisée en ce que le catalyseur est un catalyseur de décomposition de peroxyde choisi parmi l'argent et le platine et des mélanges ou composés de ceux-ci, en mélange avec du noir de carbone.

7. Particule de l'une quelconque des revendications précédentes, caractérisée en ce que la particule a un diamètre moyen allant de 0,7 mm à 4 mm et que ledit revêtement a une épaisseur de 25 à 125 microns.

8. Particule de l'une quelconque des revendications précédentes, caractérisée en ce que le liant polymère hydrophobe est un liant formé de fluorocarbone polymère.

9. Particule de l'une quelconque des revendications 1 à 5, 7 ou 8, caractérisée en ce que le catalyseur est du noir de carbone et que le liant est du polytétrafluoroéthylène, le rapport en poids du noir de carbone au liant allant de 4:1 à 1:4, de préférence de 1:1,5 à 1,5:1.

10. Procédé de préparation de particules convenant pour être utilisées en tant que matériau d'électrode selon l'une quelconque des revendications 1 à 9, caractérisé en ce qu'on forme un mélange fluide d'un catalyseur électriquement conducteur et électrochimiquement actif choisi parmi le noir de carbone, le charbon actif, le platine, l'argent ou des mélanges de ceux-ci, et d'un liant polymère hydrophobe, qu'on revêt à l'aide d'un tel mélange un support. sensiblement sphérique choisi parmi l'acier, le fer, le nickel, le platine, le cuivre, l'argent ou le graphite, qu'on fait se solidifier ledit mélange, et qu'on forme les particules ayant un diamètre moyen supérieur à 0,3 mm et jusqu'à 2,5 cm.

11. Procédé de la revendication 10, caractérisé en ce qu'on forme le mélange fluide en chauffant le liant polymère jusqu'à une température au moins aussi élevée que sa température de ramollissement, et qu'on refrodit le mélange jusqu'à une température inférieure à la température de ramollissement afin de lier le revêtement au support.

12. Procédé de la revendication 10, caractérisé en ce qu'on forme le mélange fluide en dispersant le catalyseur, le liant et le support dans un liquide, et qu'on chauffe le mélange afin de faire s'évaporer le liquide pour lier le revêtement au support.

13. Procédé de l'une quelconque des revendications 10 à 12, caractérisé en ce qu'on forme le mélange fluide en dissolvant le liant dans un solvant, et qu'on chauffe le mélange afin de faire s'évaporer le solvant pour lier le revêtement au support.

14. Procédé de l'une quelconque des revendications 10 à 13, caractérisé en ce que le catalyseur est du noir de carbone et le liant est du polytétrafluoroéthylène, le rapport en poids du noir de carbone au liant allant de 4:1 à 1:4, de préférence de 1:1,5 à 1,5:1.

15. Procédé de l'une quelconque des revendications 10 à 13, caractérisé en ce que, si on utilise une poudre métallique comme catalyseur, le rapport du catalyseur au liant est dans le domaine allant de 4:1 à 1:4 en volume, de préférence dans le domaine allant de 1:1,5 à 1,5:1 en volume.

16. Procédé de l'une quelconque des revendications 10 à 15, caractérisé en ce qu'on ajoute au mélange un agent tensioactif, de préférence un agent tensioactif non ionique.

17. Procédé de l'une quelconque des revendications 10 à 16, caractérisé en ce qu'on ajoute un second catalyseur, qui est un catalyseur de décomposition de peroxyde.

18. Procédé de la revendication 17, dans lequel la quantité totale de catalyseur dans le mélange est de 1 à 35 pour cent en poids de catalyseur de décomposition de peroxyde et de 65 à 99 pour cent en poids de noir de carbone, et de préférence de 3 à 10 et de 90 à 97 pour cent en poids.

19. Procédé pour électrolyser un électrolyte aqueux dans une cellule électrolytique ayant un compartiment anolyte avec une anode dans celui-ci et un compartiment catholyte avec un cathode dans celui-ci, lequel procédé consiste à introduire ledit électrolyte aqueux dans la cellule, à faire passer un courant électrique entre l'anode et la cathode et à récupérer les produits de l'électrolyse, caractérisé en ce qu'au moins l'une des électrodes est formée d'un matériau d'électrode comprenant une multiplicité de particules tassées selon l'une quelconque des revendications 1 à 9.

20. Procédé de la revendication 19, caractérisé en ce qu'on dispose une barrière perméable aux ions entre l'anode et la cathode.

21. Procédé de la revendication 19 ou 20, caractérisé en ce qu'on introduit dans la cathode un gaz contenant de l'oxygène.

22. Cellule électrolytique ayant un compartiment anolyte avec une anode dans celui-ci et un compartiment catholyte avec une cathode dans celui-ci, des moyens pour introduire un électrolyte aqueux dans la cellule, des moyens pour faire passer un courant électrique entre l'anode et la cathode, et des moyens pour récupérer les produits de l'électrolyse à partir de la cellule, caractérisée en ce qu'au moins l'une de l'anode ou de la cathode est formé d'un matériau d'électrode comprenant une multiplicité de particules tassées selon l'une quelconque des revendications 1 à 18.

23. Cellule de la revendication 22, caractérisée en ce que le support comprend du graphite, que le catalyseur est choisi parmi le noir de carbone, l'argent ou le platine, et que le matériau liant hydrophobe est du polytétrafluoroéthylène.

24. Cellule de la revendication 22, caractérisée en ce que le catalyseur est un mélange de noir de carbone et d'un catalyseur de décomposition de peroxyde.
